

## UNITED STATES PATENT OFFICE

2,339,340

## FUGITIVE COLORING OF YARNS

Paul Knapp, Waynesboro, Va., assignor to E. I.  
du Pont de Nemours & Company, Wilmington,  
Del., a corporation of Delaware

No Drawing. Application August 11, 1941,  
Serial No. 406,405

2 Claims.

(Cl. 8—56)

This invention relates to the fugitive coloring of filaments, yarns and threads of cellulose organic acid esters such as cellulose acetate.

By "fugitive coloring" or similar terminology used hereinafter is meant a coloration capable of substantially complete removal by a short treatment with warm dilute soap solution.

In the manufacture of certain textile products, different types of yarn are used and it is desirable to differentiate and distinguish the various yarns in order to observe the fabric construction. Accordingly, one or more of the yarns going into the fabric are fugitively colored. Dyes for this purpose are preferably of a water-soluble type which can be conveniently applied to the yarn from simple aqueous solution, and which can be readily removed from the yarn in the fabric by a moderate scouring operation without coloring or staining the other types of yarn in the fabric.

In the fugitive dyeing of cellulose acetate yarn, however, dyes which meet the preferred requirements above outlined generally do not yield satisfactory tints, and in the relatively few instances where the tints are satisfactory the fugitivity of the color is seldom all that could be desired. To cure this latter defect it has been proposed to dry the tinted yarn immediately after the application of the aqueous dye composition. However, the fugitivity required is not always obtained by this treatment under the present conditions of high speed spinning where the yarn leaving the spinning cell contains a high percentage of solvent; for example, cellulose acetate yarn spun by the evaporative method from an acetone solution and wound up at a speed of 600 yards or more per minute, may contain as much as 20% residual solvent. Coloring matter applied to this highly solvent-laden, and hence highly swollen, yarn frequently strikes in and in spite of immediate drying the yarn is sometimes more or less permanently stained.

It is, therefore, an object of this invention to provide a dyestuff which is eminently suited for the fugitive tinting of filaments, yarns and threads of organic acid esters of cellulose, such as cellulose acetate. Another object is to provide a dyestuff for the fugitive tinting of cellulose acetate which dyestuff can be easily applied to freshly spun yarn from aqueous composition to distinctively tint the same, and which can be readily removed from the yarn by moderate scouring without noticeably coloring yarns of other types with which the cellulose acetate may be associated in a fabric. Other objects will appear hereinafter.

These objects are realized by my invention which comprises applying, as the fugitive coloring material, an aqueous solution of Naphthol Green B (the ferric salt of 1-nitroso-2-naphthol-6-sodium sulfonate; Color Index No. 5) to freshly spun cellulose organic acid ester yarn.

Naphthol Green B is preferably applied at the spinning machine to freshly formed cellulose acetate yarn to the extent of from 0.05% to 0.5% based on the air dry weight of the yarn. The yarn may be simultaneously tinted and finished by dissolving the dyestuff in a suitable aqueous finish emulsion containing the usual textile finishing agents such as olive oil, sulfonated olive oil, soap, polyhydric alcohol, mineral oil, etc., and applying the composition to the yarn as it leaves the cell by a suitable roll applicator. The tint may, however, be applied quite independently of the finish by contacting the yarn with a dilute aqueous solution of the same in any suitable manner.

Even though the yarn to which the dye is applied may, and usually does, contain a very high concentration of solvent, such as 15 to 20% acetone, up to 0.5% of this dye (based on the air dry weight of the yarn) may be applied to freshly spun cellulose acetate yarn without resorting to any special procedure, for instance, such as immediately drying the yarn, a step heretofore considered essential to produce tinted yarn showing excellent fugitivity. This unusual high degree of fugitivity makes this dye outstanding for the fugitive tinting of cellulose acetate yarn before its initial windup. Although as much as 0.5% of the dye may be applied to the yarn, in general, for fugitively tinting yarn to be used in the manufacture of woven goods, substantially less than this amount is eminently satisfactory and from about 0.05% to 0.25% is preferred.

My invention is further illustrated by the following example, wherein percentages are percentages by weight.

An aqueous tint finish solution is prepared of the following composition:

|                                  | Per cent |
|----------------------------------|----------|
| Sulfonated olive oil             | 4.5      |
| Mineral oil                      | 9.0      |
| Triethanolamine oleate           | 2.0      |
| (Du Pont) Naphthol Green B conc. | 1.0      |
| Water                            | 83.5     |

Cellulose acetate yarn dry spun from an acetone solution is passed over a rotating finish applicator roll, dipping in the emulsion contained in the suitable finish trough so as to apply to the yarn

sufficient of the aqueous tint finish so that when the yarn is dried it will contain 1.5% to 4.0% of the non-volatile finish ingredients and in addition about 0.10% to 0.27% of the Naphthol Green dye. After contacting the finish applicator roll, the yarn is led over a takeup roll and onto a yarn package without any special attempt to dry the yarn, the windup being at the rate of about 600 yards per minute.

A mixed fabric is made comprising the cellulose acetate yarn so treated and viscose rayon yarn. The coloring matter in the cellulose acetate yarn is easily discharged by treating the fabric for ten minutes in an aqueous soap solution containing 0.2% sodium oleate and heated to a temperature of 70° C. Upon examination of the fabric, it will be noted that the cellulose acetate yarn has completely discharged its color and that no staining of the viscose rayon yarn has occurred. Furthermore, the short time and low temperature discharge treatment has not materially affected the luster of the cellulose acetate yarn.

The very high degree of fugitivity of Naphthol Green B, even when applied under conditions normally considered as destroying fugitivity of the dyed structure, makes this invention admirably suited for commercial use. High spinning speeds may be used with their attendant high solvent content of the yarn thus produced without sacrificing any degree of fugitivity. Furthermore, by not drying the tinted yarn, but winding the yarn into a package form while it

is still wet with the aqueous tint finish, better cake formation is secured which makes subsequent handling and unwinding more efficient with the final packaged yarn of improved quality. Since the affinity of all types of yarn for this dye is extremely poor, it may be used as a fugitive color on cellulose acetate to be combined in fabrics with any other textile yarn without causing the other yarn to be undesirably stained

10 in the process of discharging the dye from the cellulose organic acid ester yarn.

It is understood of course that my invention is not restricted to the exact conditions set out above for purposes of illustration, but comprehends all equivalents and modifications included in the spirit and terms of the following claims.

I claim:

1. Process for the fugitive coloring of filaments, yarns and threads of cellulose acetate  
20 which comprises applying to the filaments, yarns and threads of cellulose acetate a solution consisting of Naphthol Green B and water.

2. Process for the fugitive coloring of filaments, yarns and threads of cellulose acetate  
25 which comprises applying to filaments, yarns and threads of cellulose acetate up to 0.5% by weight, based on the air dry weight of the cellulose acetate, of Naphthol Green B from aqueous composition wherein water is the sole solvent for said  
30 Naphthol Green B and comprises the major portion of said composition.

PAUL KNAPP.